

Nov. 25, 1941.

A. COTÉ

2,263,614

## METHOD OF MAKING ELASTIC YARN

Filed Nov. 19, 1940



INVENTOR.  
*Arthur Cote'*  
*Sister of Bradley*

BY

ATTORNEY

## UNITED STATES PATENT OFFICE

2,263,614

## METHOD OF MAKING ELASTIC YARN

Arthur Côté, Outremont, Quebec, Canada, assignor to United States Rubber Company, New York, N. Y., a corporation of New Jersey

Application November 19, 1940, Serial No. 366,221

7 Claims. (Cl. 57—163)

This invention relates to a method of making a balanced elastic yarn comprising a rubber core having a roving cover or yarn cover placed about the core by a twisting or spinning operation.

It has been proposed heretofore to make an elastic yarn or covered rubber thread having one or more covers laid helically about the core by a winding operation in which the package of covering yarn is revolved about the rubber core as an axis to thereby wind the textile yarn about the rubber core. These core covering machines work very well but have to be specially constructed for this use, and when large quantities of elastic yarn are to be produced the aggregate cost of the many covering machines required to make such elastic yarn may run into a large sum of money.

The present invention therefore contemplates a method of making elastic yarn by a twisting or spinning operation in contrast to the winding operation just described, whereby the use of a core covering machine may be avoided and apparatus closely resembling the twisting or spinning mechanism of the textile art may be used to produce the desired elastic yarn.

It has been proposed heretofore as disclosed by the Foster Patent No. 2,024,156, Elastic yarn and process of making the same, to employ twisting or spinning mechanism to produce a single cover elastic yarn consisting of a pre-twisted rubber core having a roving cover spun about the core in a direction opposite to the twist of the core to thereby provide a balanced single cover elastic yarn.

In accordance with the disclosure of this Foster patent the pre-twisted rubber core and the textile covering material are passed between the same pair of feed rolls, to be delivered by these rolls to the twisting or spinning mechanism which serves to place the covering material about the core in helical windings.

Large quantities of highly satisfactorily elastic yarn having a stretch below 200% have been produced under this Foster patent, but it is found that the arrangement shown in the patent is not well adapted to produce a long stretch elastic yarn having a stretch considerably in excess of 200%. This is due to the fact that when the pre-twisted rubber core and textile covering material are supplied to the twisting or spinning mechanism by the same pair of feed rolls, both the cover and core are necessarily advanced by these rolls at the same speed. When this arrangement is used it is not possible to feed the covering material fast enough with respect to the rubber core to provide a sufficient length of covering material to form a long stretch elastic yarn.

The present invention therefore contemplates an important improvement in the method of the

Foster patent whereby excellent elastic yarn which is well covered and having any desired stretch up to 400% or higher may be produced upon twisting or spinning mechanism.

5 The method of the present invention is based largely upon the discovery that important advantages are obtained, and a much greater control over the stretch characteristics and other properties of the elastic yarn being produced are secured if the pretwisted rubber core and covering material are advanced toward the twisting mechanism by independent means, so that one may be advanced at a faster speed than the other. By feeding the covering material to the 10 covering point at a different speed from that of the rubber core sufficient covering material can be supplied to the rubber core to provide for any desired range of stretch.

One field in which large quantities of elastic 20 yarn or covered rubber thread are used is that of knitting in which it is used as the yarn that is knitted into the fabric, and also as the yarn which is laid-in along the courses of the fabric. Elastic yarn which is knitted into a fabric usually has a stretch below 200%, whereas laid-in elastic yarn usually has a stretch considerably in excess of 200%. There are also other fields in which a long stretch elastic yarn is required.

Prior to the present invention it was not possible to make good elastic yarn by a spinning or 25 twisting operation having a stretch long enough to cause it to be well adapted for use as a laid-in elastic yarn in a knitted fabric. Through the present invention elastic yarn can be made by a spinning operation with sufficient stretch 30 for use in this laid-in field and in various other fields where a long stretch elastic yarn is required.

The method of the present invention may be 35 employed to produce by a spinning operation an elastic yarn consisting of a pre-twisted rubber core having a roving spun thereupon as a cover, or it may be employed to produce by a spinning 40 operation an elastic yarn having a textile yarn applied helically about the rubber core as a cover. In either case, by supplying the rubber core to the spinning mechanism at one speed and the covering material at a different speed, a 45 much greater range of stretch can be secured than could be obtained heretofore when elastic 50 yarn was produced by a twisting or spinning operation.

In carrying out the present invention the pre-twisted rubber thread is advanced to the twisting or spinning mechanism from one source of supply and the covering material is advanced to this mechanism from a separate source of supply. In some cases it may be desirable to use one pair of power driven feed rolls to advance the rubber core to the spinning position

and a separate and independently operated pair of power driven rolls for advancing the covering material to the spinning position. In other cases it will be sufficient to provide only one pair of power driven feed rolls which may be employed, for example, to pull the covering material towards the spinning apparatus at a predetermined speed while the rubber core may be pulled direct from its source of supply by the spinning spindle. The essential requirement is that provision be made for supplying the covering material to the spinning position at a higher linear speed than the rubber core, or at a lower linear speed than the rubber core, as may be required by the particular elastic yarn being produced.

The above and other features of the invention will be further understood from the following description when read in connection with the accompanying drawing illustrating good practical forms of mechanism for carrying out the present method.

In the drawing:

Fig. 1 is a conventional diagrammatic view of one form of mechanism for delivering a drafted roving to spinning mechanism adapted to spin the roving about a pre-twisted rubber thread to form an elastic yarn.

Fig. 2 is a somewhat similar view of mechanism for producing an elastic yarn having a textile yarn applied helically about the rubber core as a cover.

Fig. 3 differs from the construction of Fig. 2 only in that the cover is formed of two textile yarns in Fig. 3 and of one textile yarn in Fig. 2.

Fig. 4 is an enlarged view of an elastic yarn produced upon the apparatus of Fig. 1.

Fig. 5 is a similar view of an elastic yarn produced upon the apparatus of Fig. 2, and

Fig. 6 is a similar view of an elastic yarn produced upon the apparatus of Fig. 3.

Various forms of apparatus may be employed to carry out the method of the present invention, and while different types of twisting or spinning mechanism may be used to twist the covering material and rubber core together, to thereby produce the elastic yarn, it is preferred to employ the well known type of ring and traveller spinning mechanism.

In the apparatus shown in Fig. 1 the pre-twisted rubber core 10 is conveniently supplied to the spinning mechanism from a spool 11. This rubber core may be any suitable elastic thread formed of rubber or rubber like material having the desired stretch, durability and other required properties, and it preferably has a high twist imparted thereto before it is wound on to the package 11. This rubber thread may be as fine as ".01" in diameter or finer, or as large as desired.

It is desirable to control the rate at which the rubber thread 10 is unwound from the spool 11. This is readily accomplished by supporting the spool so that it will rest by gravity upon the power driven roll 12 to thereby rotate the spool 11 so as to unwind the rubber thread therefrom at a uniform speed irrespective of the size of the package. The arms 13 pivoted at 14 may be provided to support the spool 11 in engagement with the roll 12.

The covering material shown in Fig. 1 comprises the roving 15 supplied by the bobbin 16. This roving is preferably drafted in a well known manner by the pairs of drafting rolls 17, 18 and 19 which serve to attenuate the roving in the

direction in which its travels so that it leaves the rolls 19 as an untwisted or slightly twisted strand of loosely aggregated fibers.

The advancing rubber thread 10 and drafted roving 15 converge towards each other to a meeting point somewhat near the pigtail 20 disposed above and in axial alignment with the spinning spindle 21. At this meeting point the rubber thread 10 and textile strand 15 are brought into side by side longitudinal relation with each other and are then immediately united by a yarn plying operation imparted thereto by the spindle 21. The united rubber thread and roving then pass downwardly through the traveler 22 upon the ring 23 and inwardly to be wound about the spindle 21 to form the package 24 of elastic yarn. The spinning spindle 21 may be driven by the belt 25 or by other means as desired.

If a balanced elastic yarn is to be produced as herein contemplated it is important that the spindle 21 be rotated in a direction to remove part of the twist previously imparted to the rubber thread 10, so that the operation of spinning the cover about the rubber core will serve to remove part of the twist previously imparted to the core, to thereby provide an elastic yarn in which the helical windings of the cover in one direction serve to balance the twist of the core in the opposite direction as will be apparent from Fig. 4.

The speed at which the rolls 19 are operated will determine the speed at which the covering material 15 is delivered to the covering point, and a pair of power driven feed rolls 26 may be provided to deliver the rubber thread 10 to the covering point at a speed either faster or slower than that at which the covering material is delivered, depending upon the requirements of the elastic yarn being produced.

In the construction of Fig. 1 in which a roving is employed as the covering material it is desirable that the rubber thread and covering material shall converge towards each other at substantially equal angles as shown. This will give some of the twist imparted to the combined core and cover an opportunity to pass upwardly beyond the pigtail 20 so as to impart a few twists per inch to the drafted roving and thereby increase its strength before it reaches the rubber thread 10. In this manner an elastic yarn having a stronger roving cover as well as a greater stretch than heretofore may be produced.

In some cases it may be desirable to produce an elastic yarn having a cover of textile yarn in place of the roving of Figs. 1 and 4. In this case the apparatus of Fig. 2 may be employed where in the same type of spinning mechanism of Fig. 1 is provided and the pre-twisted rubber thread 10' may be supplied from a let-off package 11' the same as in Fig. 1. In this construction of Fig. 2 the textile yarn 27 forming the cover for the elastic yarn may be supplied from a cone 28. As this yarn 27 leaves its supply cone it preferably is drawn through a tension device 29 adapted to exert a slight tension thereupon, and is preferably pulled forward by the power driven feed rolls 30 to pass downwardly to the pigtail 20.

In the construction of Fig. 2 it should be noted that the feed rolls 26 of Fig. 1 have been omitted. This is because it is found that the feed rolls 26 are not necessary since the tension of the rubber thread and rate of feed of the same can be controlled simply by employing the driving roll 12 to control the speed at which the rubber thread 10' is unwound from its package 11. It will be

TABLE II.—Roving covered elastic yarn

|    |                                                    | A                         | B                         | C                         |
|----|----------------------------------------------------|---------------------------|---------------------------|---------------------------|
| 5  | 1 Core—rubber thread.....                          | 100's.....                | 100's.....                | 100's.....                |
| 2  | Cover—roving.....                                  | 4 hank 2 ends cotton..... | 4 hank 3 ends cotton..... | 4 hank 3 ends cotton..... |
| 3  | Elongation—elastic yarn.....                       | 125%.....                 | 220%.....                 | 330%.....                 |
| 4  | Yards per pound—elastic yarn normal condition..... | 7400.....                 | 3940.....                 | 3150.....                 |
| 10 | Length of (relaxed) core in 1 yard.....            | 23.8".....                | 31.5".....                | 39.6".....                |
| 15 | Length of cover in 1 yard*.....                    | 93.6".....                | 133.2".....               | 204.0".....               |
| 6  | Bare core—by weight.....                           | 41.2%.....                | 31.2%.....                | 30.0%.....                |
| 7  | Cover—by weight.....                               | 58.8%.....                | 68.6%.....                | 70.0%.....                |
| 8  | Gauge—elastic yarn relaxed.....                    | .014.....                 | .022.....                 | .028.....                 |

\*Theoretical length.

The large excess in the length of cover relative to the length of core in the above tables is readily secured by feeding the cover to the twisting mechanism faster than the core as herein contemplated.

Having thus described my invention, what I claim and desire to protect by Letters Patent is:

1. The method of making a balanced single cover elastic yarn which consists in delivering a pre-twisted rubber thread and a covering yarn along separate paths and at independently controlled speeds to a meeting point adjacent twisting mechanism, to thereby bring the rubber thread and a predetermined different length of said yarn into side by side longitudinal relation, and then twist them together by a yarn plying operation in a direction to remove part of the twist previously imparted to the rubber thread and place one about the other so that as the thread assumes a central position the yarn will lie helically about the rubber thread as a cover.
2. The method of making a balanced single cover elastic yarn which consists in delivering a pre-twisted rubber thread and a textile strand along separate paths and at independently controlled speeds to a meeting point adjacent twisting mechanism, to thereby bring the rubber thread and a predetermined different length of said strand into side by side longitudinal relation, and then twist them together by a yarn plying operation in a direction to remove part of the twist previously imparted to the rubber thread and place one about the other so that as the thread assumes a central position the strand will lie helically about the rubber thread as a cover.

3. The method of making a balanced single cover elastic yarn which consists in supporting in feeding relation to twisting mechanism a source of textile covering yarn and a pre-twisted rubber thread, exerting an independently operated pulling force on the textile yarn and thread to advance them at independent speeds towards a meeting point, bringing them together into side by side longitudinal relation, and then twisting them together by a yarn plying operation in a direction to remove part of the twist previously imparted to the rubber thread and place one about the other so that as the thread assumes a central position the strand will lie helically about the rubber thread as a cover that balances the twist of the thread.

4. The method of making a substantially balanced single cover elastic yarn which consists in supporting in feeding relation to twisting mechanism a source of textile covering strand and a pre-twisted rubber thread, operating the twisting mechanism to exert an advancing pull on the strand and thread, exerting a further ad-

TABLE I.—Yarn covered elastic yarn

|   |                                                    | A                  | B                  | C                  |
|---|----------------------------------------------------|--------------------|--------------------|--------------------|
| 1 | Core—rubber thread.....                            | 100's.....         | 100's.....         | 100's.....         |
| 2 | Cover.....                                         | 22/1/1 cotton..... | 22/1/1 cotton..... | 22/1/1 cotton..... |
| 3 | Elongation—elastic yarn.....                       | 200%.....          | 280%.....          | 400%.....          |
| 4 | Yards per pound—elastic yarn normal condition..... | 3820.....          | 3640.....          | 2740.....          |
| 5 | Length of (relaxed) core in 1 yard.....            | 25.2".....         | 26.5".....         | 36".....           |
| 6 | Length of cover in 1 yard.....                     | 124.7".....        | 158.0".....        | 207.9".....        |
| 7 | Bare core—by weight.....                           | 27.3%.....         | 26.0%.....         | 25.0%.....         |
| 8 | Cover—by weight.....                               | 72.7%.....         | 74.0%.....         | 75.0%.....         |
| 9 | Gauge—elastic yarn relaxed.....                    | .019.....          | .0225.....         | .027.....          |

vancing pull upon said strand independently of said thread to thereby advance the strand faster than the thread and bring them into side by side longitudinal relation, and then twist them together by a yarn plying operation in the opposite direction to the twist previously imparted to the rubber thread to place one about the other so that as the thread assumes a central position the strand will lie helically about the rubber thread as a cover.

5. The method of making a substantially balanced single cover elastic yarn which consists in supporting in feeding relation to twisting mechanism a source of textile covering strand and a pre-twisted rubber thread, exerting an advancing pull on the strand and exerting a separate and independent advancing pull on the thread to advance one faster than the other, bringing them together into side by side longitudinal relation and twisting them together by a yarn plying operation in the opposite direction to the twist previously imparted to the rubber thread to place one about the other so that as the thread assumes a central position the stand will lie helically about the rubber thread as a cover.

6. The method of making a substantially balanced single cover elastic yarn which consists in supporting in feeding relation to twisting mechanism a source of textile covering strand and a pre-twisted rubber thread, providing sepa-

rate and independent power driven feed means for the thread and strand operable to advance the thread and strand at different relative speeds towards a meeting point, bringing them together into side by side longitudinal relation, and then twisting them together by a yarn plying operation in a direction to remove part of the twist previously imparted to the rubber thread and place one about the other so that as the thread assumes a central position the yarn will lie helically about the thread as a cover.

7. The method of making a balanced single cover elastic yarn which consists in supporting in feeding relation to twisting mechanism a plurality of packages of textile yarn and a supply of pre-twisted rubber thread, exerting an advancing pull on each yarn and exerting a separate and independent advancing pull on the rubber thread to advance one faster than the other, bringing them together into side by side longitudinal relation, and then twisting them together by a yarn plying operation in the opposite direction to the twist previously imparted to the rubber thread to thereby decrease the twist of the rubber thread and place one about the other so that as the thread assumes a central position the yarns will lie helically about the thread so as to balance its twist and hold the thread stretched.

ARTHUR COTÉ.